

## UNITED STATES PATENT OFFICE

2,632,003

TREATMENT OF STICKLAC TO OBTAIN  
THEREFROM SEEDLAC

Robert Hutchison Turnbull, Calcutta, India

No Drawing. Application December 14, 1951, Se-  
rial No. 261,758. In India July 26, 1950

11 Claims. (Cl. 260—107)

1

The invention is for improvements in and relating to the treatment of sticklac whereby to obtain therefrom seedlac. The invention has for a particular object so to treat the poorer qualities of sticklac, such as those known to the trade as Siam sticklac, as to obtain therefrom good quality seedlac equivalent, for example, to that known in the trade as Kusmi seedlac.

Sticklac (i. e. the original form in which the lac is gathered) contains the lac deposits mixed with sticks or twigs from which it derives its name, and also foreign matter such as dirt, dust, sand, albumen, nitrogen and a relatively high quantity of colouring matter which is more particularly a red dye. Seedlac is the material obtained after refining or purifying the raw sticklac, the treatment having for object to remove the sticks, twigs, dirt and other impurities and as much as possible of the colouring matter, so as to obtain a product which will require as low a bleach consumption as possible in order to obtain a commercially useful product. Qualities of seedlac used for commercial purposes are generally determined and classified by their nitrogen and bleach numbers and content of impurities.

It is already known to treat sticklac to produce seedlac by various processes having for object the removal of the impurities and colouring matter aforesaid, the steps involved comprising a preliminary grinding and washing of the sticklac, the treatment of the ground and washed material with one or more chemicals to remove the colouring matter, and a further washing and drying.

The present invention provides an improved process whereby the impurities and colouring matter are more efficiently removed than hitherto and there is obtained a seedlac which has a lower nitrogen content, a lower content of impurities and an improved bleach consumption and rate of bleach as compared to seedlac hitherto obtained from similar quality sticklac.

The process of the invention is based primarily on the step in the treatment of sticklac to obtain seedlac, which consists in subjecting the said sticklac to the action of ammonium sulphate for the purpose of removing colouring matter, albuminous matter and other foreign matter from the lac grains.

In particular and preferably, the process of treatment according to the invention comprises the successive steps of grinding and washing the sticklac, subjecting the same to the action of ammonium sulphate as aforesaid and thereafter following the said ammonium sulphate treatment

2

with conventional or special washing and/or other treatments to recover the refined lac grains.

The advantageous results obtained in the separation of foreign matter from the lac grains by the use of ammonium sulphate in the method of the invention are believed to be due to the faculty of ammonium sulphate to promote its adsorption by the sticklac. It has been found that ammonium sulphate is readily dissociated and, when used in the method of the invention, the whole ionic system is so disturbed that all foreign matter is readily released from contact with the sticklac and so separates out from the system by alteration of surface tension and is precipitated.

15 The ammonium sulphate treatment according to the invention is effected with the ammonium sulphate in the form of an aqueous solution and the complete process steps comprise grinding and washing the sticklac with water, recovering the ground and washed lac material, subjecting the same in a ball mill or the equivalent to the action of a solution of ammonium sulphate, separating the treated lac from the solution containing the impurities removed from the lac 20 grains, repeating the milling operation one or more times, recovering the treated lac, subjecting the same to one or more washings, with a solution of common salt, further washing the treated lac with water, and drying the final 25 product.

30 Preferably, the grinding treatment in the ball mill is effected with at least a 0.5% solution of ammonium sulphate over a period of about four to five hours and the millings are repeated until 35 the wash water shows no further signs of colouring matter. For the washing with common salt, a solution of about 1.2 specific gravity is preferably used and, after stirring, settling is effected whereby the dirt and the impurities fall to the

40 bottom and the lac floats to the top of the solution. The clean lac is then separated from the liquid residue and further washing with common salt solution is repeated one or more times. The washed lac is then subjected to a combined centrifugal and filter action while being further 45 washed with water, whereafter it is dried in the centrifugal machine, followed by air drying.

In order that the invention may be more fully understood, a detailed example thereof will now 50 be given in the following by way of illustration.

Example.—Siam sticklac is roughly ground in a disintegrator to pass through a 10 mesh sieve, or coarser. The ground material is then sieved on an 80 mesh sieve so as to get rid of the fine dust 55 of foreign character and the sand. Before grind-

ing roughly, any bare sticks or twigs are first removed by hand.

The sticklac so ground is placed in an open receptacle, such as a tub, and thoroughly washed with water, by mixing with a beater, such as a wooden stick. This removes a quantity of the red colouring matter or dye. After mixing thoroughly, the sticklac is allowed to settle and the wash water is removed by syphoning, passing the syphoned water through an 80 mesh sieve to catch any particles of sticklac. This washing is continued until all the red dye is removed by the water which generally takes about three or four washings, depending on the nature of the sticklac.

The washed sticklac is then transferred to an 80 mesh sieve to enable the water to be drained off. The sticklac is then collected and placed in a porcelain ball mill, one third of which is already filled with porcelain balls of about one inch in diameter. A quantity of 0.5% ammonium sulphate solution is added to fill the ball mill up to about two thirds of its capacity. In some instances, the use of about 1.0% ammonium sulphate solution may be required, depending upon the quality of the sticklac. The ball mill is then rotated at a speed of about 45 to 50 revolutions per minute for a period of about four to five hours. After such milling, the ball mill is removed from its carriage and the sticklac allowed to settle. The coloured (red) water is then removed by syphoning and passed through an 80

before all the foreign matter is removed from the sticklac. The salt solution is then recovered by passing the same through a filter press and used again for washing purposes. This is easily observed when no further precipitation of impurities is seen.

10 The washed sticklac is then transferred to a centrifugal with perforated sides, over which a good filter cloth is placed. Then, when the centrifugal is running, the seedlac is washed with water until the wash water is free from chlorides, as ascertained by chemical test. As soon as such result is achieved, the sticklac is dried by means of a centrifugal machine and finally air dried in 15 perforated shelves, covered with gunny.

20 In carrying the above-described process of the invention into practice, a horizontally-driven centrifugal machine is preferably employed, which enables the sticklac under treatment to be continuously fed and washed in one operation.

25 By way of example, it is indicated that the average impurities content of sticklac treated by the method of the invention and as determined by standard methyl or ethyl alcohol tests is found to be between about 0.36% and 1.20%, which is considerably lower than the impurities content obtained with previously known methods of treatment. Further, on six samples of poor quality Siam sticklac A, B, C, D, E and F treated by the 30 process according to the invention, the following results were obtained in respect of nitrogen content and bleach tests.

| Samples                  | Nitrogen, percent | ccs. of std. bleach sol. reqd. for 30 grams of lac | Colour of bleach sol. compared with standard        | Rate of bleach compared with standard   |
|--------------------------|-------------------|----------------------------------------------------|-----------------------------------------------------|-----------------------------------------|
| A=145 grs.....           | 0.04              | 35                                                 | Somewhat greyer.....                                | Similar.                                |
| B=247 grs.....           | 0.06              | 65                                                 | More yellow than standard, and also than C.         | Considerably slower.                    |
| C=275 grs.....           | 0.05              | 55                                                 | Somewhat more yellow than standard and also than E. | Considerably slower but less so than B. |
| D=250 grs.....           | 0.07              | 60                                                 | Similar to C.....                                   | Similar to C.                           |
| E=222 grs.....           |                   | 55                                                 | Very slightly yellower.                             | "Do."                                   |
| F=185 grs.....           |                   | 60                                                 | Similar to B.....                                   | Similar to B.                           |
| Fine Kusmi standard..... | 0.15              | 55                                                 |                                                     |                                         |

mesh sieve to collect any escaping sticklac. The process is then repeated with three or four millings until the wash water shows no further signs of red colour.

When this stage is reached, the sticklac is removed to a separator, a preferred form of which has a rectangular open top, with square sides, which sits on a foundation of four sloping sides and which is provided with two glass windows, one on either side, for viewing the operation of washing. At the base is fixed a tube with a valve for drawing off the wash water. To the sticklac, now in the separator, is added a quantity of common salt solution of 1.2 specific gravity. The whole is well mixed with a beater, such as a wooden stick, and then allowed to settle until the salt solution becomes clear. At this stage, all the foreign matter, such as dirt and foreign organic matter, as well as most of the albuminous matter, falls to the bottom, while the sticklac goes to the top of the liquid. The whole of the salt solution is then drawn off, along with the residues which are at the bottom of the separator, leaving the clean sticklac in the separator. A further quantity of the same strength of salt solution is then added to the separator, and the same washing process repeated. Three or four washings with salt solution may be necessary

50 The bleach tests were carried out employing as standard a sample of fine Kusmi standard 1937. The directions followed were those usual for standard Kusmi seedlac for all samples except sample A where, owing to the low bleach consumption, the method adopted was to add 25 ccs. of bleach solution to a total volume of 275 ccs., so that the 240 cc. aliquot taken next day corresponded to 20 cc. of bleach solution and 30 grams of seedlac. The colour of all samples after bleaching was found generally to be a pale yellowish-cream.

55 It will be seen that by means of the invention it is possible to treat poor quality sticklac to obtain therefrom a quality of seedlac which is comparable with, or even superior to, fine Kusmi standard seedlac in respect of nitrogen and impurities content and bleach consumption. It will be understood, however, that the invention is not limited to the specific details thereof which have been given above by way of example and that many modifications of the same may be made within the scope of the appended claims.

I claim:

60 1. In the treatment of sticklac to produce seedlac, the improvement which comprises the step of subjecting the sticklac to the action of ammonium sulphate in aqueous solution to cause sepa-

ration of colouring matter, albuminous matter and other foreign matter from the lac grains.

2. In the treatment of sticklac to produce seedlac, the improvement which comprises the steps of subjecting the sticklac to the action of an aqueous solution of ammonium sulphate to cause colouring matter, albuminous matter and other foreign matter to separate from the lac grains and washing with an aqueous solution of common salt.

3. A process for the treatment of sticklac to produce seedlac, which comprises grinding and washing the sticklac, subjecting the ground and washed sticklac to the action of ammonium sulphate in aqueous dilute solution to cause colouring matter, albuminous matter and other foreign matter to separate from the lac grains, removing the separated matter, and washing and drying the resultant treated lac.

4. A process for the treatment of sticklac to produce seedlac, which comprises grinding and washing the sticklac with water, recovering the ground and washed lac material, milling said lac material in admixture with an aqueous dilute solution of ammonium sulphate, recovering the so-treated lac material from said mixture after milling, washing said lac material with a solution of common salt, and then washing with water and drying.

5. In the treatment of sticklac to produce seedlac, the improvement which comprises the step of subjecting the sticklac to the action of ammonium sulphate in the form of an at least 0.5% aqueous solution to cause colouring matter, albuminous matter and other foreign matter to separate from the lac grains.

6. In the treatment of sticklac to produce seedlac, the improvement which comprises the step of subjecting the sticklac to the action of ammonium sulphate in the form of an at least 0.5% aqueous solution over a period of about four to five hours, to cause colouring matter, albuminous matter and other foreign matter to separate from the lac grains.

7. A process for the treatment of sticklac to produce seedlac, which comprises grinding and washing the sticklac with water, recovering the ground and washed lac material, milling said lac material in admixture with an at least 0.5% aqueous solution of ammonium sulphate over a period of about four to five hours, recovering the so-treated lac material from said mixture after milling, washing said lac material with a solution of common salt, and then washing the treated lac with water and drying the final product.

8. In the treatment of sticklac to produce seedlac, the improvement which comprises the

steps of subjecting the sticklac to the action of ammonium sulphate in the form of an at least 0.5% aqueous solution over a period of about four to five hours, to cause colouring matter, albuminous matter and other foreign matter to separate from the lac grains, and washing the treated lac with a common salt solution of about 1.2 specific gravity.

9. A process for the treatment of sticklac to produce seedlac, which comprises grinding and washing the sticklac, subjecting the ground and washed sticklac to the action of an aqueous dilute solution of ammonium sulphate to cause colouring matter, albuminous matter and other foreign matter to separate from the lac grains, removing the separated matter and washing the treated lac with a common salt solution of about 1.2 specific gravity and drying the resultant treated lac.

10. In the treatment of sticklac to produce seedlac, the improvement which includes the steps of subjecting the sticklac to the action of an aqueous dilute solution of ammonium sulphate to cause colouring matter, albuminous matter and other foreign matter to separate from the lac grains, washing the treated lac with a common salt solution, and subjecting the treated lac to a combined centrifugal and filter action while being washed with water, whereafter it is dried by centrifuging, followed by air drying.

11. A process for the treatment of sticklac to produce seedlac, which comprises grinding and washing the sticklac with water, recovering the ground and washed lac material, milling said lac material in admixture with an at least 0.5% aqueous solution of ammonium sulphate over a period of about four to five hours, recovering the so-treated lac material from said mixture after milling, washing said lac material with a solution of common salt of about 1.2 specific gravity, and finally subjecting the treated lac to a combined centrifugal and filter action while being washed with water, whereafter it is dried by centrifuging, followed by air drying.

ROBERT HUTCHISON TURNBULL.

#### REFERENCES CITED

The following references are of record in the file of this patent:

#### UNITED STATES PATENTS

| Number    | Name    | Date         |
|-----------|---------|--------------|
| 1,644,491 | Rawolle | Oct. 4, 1927 |

#### FOREIGN PATENTS

| Number  | Country       | Date          |
|---------|---------------|---------------|
| 103,006 | Great Britain | Feb. 14, 1917 |
| 188,296 | Great Britain | May 7, 1923   |